

April 16, 1963

A. W. PESCH

3,085,927

PROCESS FOR PREPARATION OF FIBERS HAVING  
DIFFERING CHARACTERISTICS

Filed Nov. 16, 1960

2 Sheets-Sheet 1



FIG. 1



FIG. 2

INVENTOR  
ANTHONY W. PESCH  
BY *Robert S. Sauborn*  
ATTORNEY

April 16, 1963

A. W. PESCH

3,085,927

PROCESS FOR PREPARATION OF FIBERS HAVING  
DIFFERING CHARACTERISTICS

Filed Nov. 16, 1960

2 Sheets-Sheet 2



FIG. 3

INVENTOR.  
ANTHONY W. PESCH

BY  
*Robert S. Sanborn*

ATTORNEY

1

3,085,927

**PROCESS FOR PREPARATION OF FIBERS HAVING DIFFERING CHARACTERISTICS**

Anthony W. Pesch, Daphne, Ala., assignor to International Paper Company, New York, N.Y., a corporation of New York

Filed Nov. 16, 1960, Ser. No. 69,728  
5 Claims. (Cl. 162—55)

This invention relates to the manufacture of cellulosic pulp, and more particularly to a process for separation of the pulp fibers into fractions having differing characteristics.

It is known that the differences between the characteristics of springwood (also called early wood) and of summerwood (also called late wood) produce marked differences in the properties of paper made from wood pulp in accordance with the variation in the proportion of springwood and summerwood in the pulp logs being used as the raw stock for the pulp.

Every tree, at least in the non-tropical zones, has annual rings which are distinctive increments of annual growth. Each annual ring consists of a portion of springwood which is that part of the annual growth which occurs early in the growing season, and a portion of summerwood which is that portion of the growth which occurs later in the season.

Generally speaking, the woods of the Northern States and Canada, particularly the softwoods or coniferous woods, have a comparatively larger amount of springwood and a comparatively smaller amount of summerwood because of the long northern winters and comparatively short summers, while the trees of the Southern States have a higher proportion of summerwood because of the longer growing season of the warmer climate.

For a given species of tree the proportions of springwood and summerwood may vary to such an extent under different growing conditions that the variation in the characteristics and properties of the paper produced from the tree is greater under identical manufacturing conditions than the variation in papers produced from two different species under different manufacturing conditions. A paper produced from a northern tree having a comparatively low amount of summerwood usually has markedly different properties from a paper produced from a southern tree of the same species or genus having a comparatively high proportion of summerwood. Likewise, papers produced from species having a higher springwood content vary from those produced from different species having a higher summerwood content. These differences are demonstrable by standard test procedures.

Such papers may, for convenience herein, be designated and distinguished as springwood papers and summerwood papers. Springwood pulps and papers, other things being equal, have less freeness, bulk, tear strength, air permeability (i.e. higher densometer or porosity test reading) and greater bursting strength (Mullen test), smoothness, fold, tensile strength and printability than summerwood paper, while the latter for many purposes has desirably greater bulk and tear strength.

While in general these facts have been known, no one, as far as known, has been able to take advantage of the differences in characteristics between springwood and summerwood of the same or different species of trees to produce papers having predetermined characteristics under commercial conditions by precisely controlling the proportions and manner of application of pulp from springwood and summerwood fibers. The best that has been done prior to this invention is to determine roughly that pulp logs from given tree species growth under given conditions in particular locations have respectively greater

2

or lesser proportions of springwood and summerwood, and to try to schedule the flow of pulp logs into and from the wood yard accordingly.

The difficulty inherent in separation and use of springwood and summerwood fibers from a given log is that since the components are thin and alternate, it is commercially impractical to separately remove the alternate thin springwood and summerwood layers from the log. This has been done if at all only on a laboratory basis and in minute quantities. Nevertheless it is highly desirable to be able to separate the springwood fibers from the summerwood fibers of a given batch of raw stock, and to handle and apply them separately or in combination in predetermined proportions in the paper making operation.

My invention accordingly consists in the appreciation of the advantages to be gained in the paper making art by using springwood and summerwood fibers in predetermined proportions and also separately, in the concept that this can be achieved by separating the two types of fiber from each other in the pulp or in the formation of the pulp, either virgin stock such as from logs and chips or re-pulped stock from waste paper and the like, in the perception of certain differing properties, among others, of springwood and summerwood fibers which can be used for such separation, and in the discovery of a process and means which makes use of these differing properties and characteristics for such separation economically on a commercial scale, as more fully hereinafter set forth in connection with the drawings, in which:

FIG. 1 is a photomicrograph of a cross section of a tree or pulp log of a typical coniferous wood or softwood, taken at the junction of two annual growth rings showing some of the differences in the characteristics of the springwood and the summerwood;

FIG. 2 is a photomicrograph showing the fibers in a typical example of softwood kraft pulp; and

FIG. 3 is a schematic drawing of one type of apparatus which may be used in the separation of cellulosic springwood and summerwood fibers.

In the drawings, FIG. 1 is a microscopic sample of a piece of softwood 1, in this case yellow pine, which may normally be used in making cellulosic pulp for the manufacture of paper and of cellulose derivatives. It shows that any such piece of wood which may be, for instance, a chip used in making chemical pulp, contains springwood fibers 2 and summerwood fibers 3 with a clearly distinguishable line of demarcation 4 between them at the junction of two annual growth rings. Both types of fibers are generally tubular and hollow. The springwood fibers 2 have comparatively thinner walls 5 and comparatively larger openings called lumens 6, and the summerwood fibers 3 have comparatively thicker walls 7 and comparatively smaller lumens 8.

In FIG. 2 the springwood fibers 2 and the summerwood fibers 3 are shown intermixed in a water pulp slurry after the wood has been digested as by cooking with the sulphate or kraft process and the fibers have been separated so that they are interspersed helter skelter. It can be seen that the summerwood fibers 3 have a more condensed appearance and structure as the result of the thicker walls 7 and smaller lumens 8, giving the dark thin appearance, while the springwood fibers 2 appear wider, with thinner walls and are lighter in appearance. The flattened appearance of the springwood fibers 2 in FIG. 2 is due to the fact that in some of the later stages of pulping due to beating and the like, these fibers have, to some extent, collapsed and become flatter in section, nevertheless retaining the essential characteristics above described.

The material of the walls 5 and 7 of both the springwood and the summerwood fibers 2 and 3 is relatively pure cellulose which has an actual specific gravity of ap-

proximately 1.6. But after the wood has been defiberized into pulp with the fibers suspended in water in typical pulp stock, the lumens or openings 6 and 8 of both types of fiber become at least partially filled with water and in this condition the springwood fibers 2 have an apparent specific gravity which is less than the apparent specific gravity of the summerwood fibers 3. That is to say, they are "lighter" when in water.

I have discovered that the differences in apparent specific gravities of the springwoods and summerwoods are sufficient so that starting with any typical pulp stock after digestion, the mixture of the types of fibers under discussion can be separated into fractions consisting essentially of springwood having a comparatively lower apparent specific gravity and summerwood having a comparatively higher apparent specific gravity.

I have also discovered that the fractionation process is favorably influenced by the fact that due to the less compact shape of the springwood fibers they tend to sink more slowly in water than the summerwood fibers which have a more compact shape, as previously described.

There are various ways to accomplish the separation by taking advantage of these differences in apparent specific gravity and sinking rate.

One example of a preferred type of apparatus is diagrammatically illustrated in FIG. 3. It consists of at least one hydrocyclone 15 of the general type used for separation of ore components of different specific gravities, as described in United States Patent No. 2,648,433 and as also used for separation of dirt from pulp, as shown in United States Patent No. 2,878,934. Such a hydrocyclone may be particularly adapted and improved for the particular purpose of efficient pulp fractionation according to the present invention, but the details of such adaptation are not herein particularly described and claimed since the scope of the invention, as presently claimed, includes the practice of the process by any one of several types of apparatus.

A typical hydrocyclone 15 has a hollow, at least partly conical, chamber 16 having a base end 18 and an apex end 20. Generally speaking, the material to be separated is pumped in slurry form tangentially through a line 22 into the chamber 16 thereafter spiralling toward the apex end 20 of the conical chamber 16 in circles of decreasing diameter and with increasing angular velocity. As a result, two concentric vortices form creating a central air column. The heavier constituent of the slurry is thrown by centrifugal force into the outer vortex and the lighter constituents are forced into the inner vortex. The lighter constituents travel upwardly along the inner vortex and leave the chamber 16 through a line 24 connected to an orifice at the base end 18 while the heavier constituents travel downwardly in the outer vortex and leave the chamber 16 through a line 26 from the apex end 20, thereby classifying the different constituents. In FIG. 3 the original pulp to be fractionated according to the invention is tangentially introduced to the chamber 16 through the line 22, and in accordance with the above summarized principle of operation the component having more than the original proportion of springwood leaves the chamber through the line 24 while the component having more than the original proportion of summerwood leaves the chamber through the line 26.

For many purposes in the practice of the invention, the use of a single hydrocyclone 15 is sufficient. As long as the proportions of springwood and summerwood fibers produced in the lines 24 and 26 respectively are measurably higher than they were in the original pulp slurry introduced in the line 22, the fractionation thereby achieved for use in paper making in predetermined amounts or proportions is within the scope of the claims.

Since complete separation into fractions containing only springwood and only summerwood respectively is probably only theoretical, the degree of separation to be achieved is primarily a matter of mechanical efficiency.

In some cases the use of one hydrocyclone 16 may not achieve the desired degree of efficiency for the purposes intended and in such instances more than one hydrocyclone may be used as illustrated. In such case the pulp slurry containing the higher proportion of springwood in the line 24 is introduced at 28 into the hydrocyclone 15a and the fraction leaving the latter through the line 30 contains a still higher proportion of springwood.

The slurry containing the higher proportion of summerwood in the line 26 may be introduced tangentially through the line 32 to another hydrocyclone 15b and the pulp slurry leaving the latter through the line 34 contains a still higher proportion of summerwood. Further refinement of the fractionation may be carried out by the use of additional hydrocyclones in series, and the slurries leaving the hydrocyclones 15a and 15b through the lines 36 and 38 respectively may be used separately on separate paper machines, applied separately through separate headboxes on the same paper machine, combined in predetermined proportions and used on a paper machine, recycled to the system, or used in any other manner in which the fractionation of the invention is advantageous.

The hydrocyclones used as described either singly or in series may also be connected in parallel batteries to increase the volume for fractionation in commercial quantities as for use in preparing pulp for large paper machines or for a number of paper machines.

Other fractionation systems can be used, for instance, quiet and flow settlement system tanks or sluice boxes which are well known for use in the separation of components of materials such as ores having different specific gravities and other characteristics which influence sinking or settlement time.

The pulp fractions of springwood and summerwood fibers can be combined and proportioned in a predetermined manner to combine desirable properties and characteristics and to reduce undesirable properties and characteristics in the paper to be produced for the purposes intended.

One specific example of the application of the invention is in the production of kraft liner board for use in making the face sheets between which the corrugated medium is sandwiched in the production of sheet stock for corrugated containers. Such a liner board is improved if it has good bulk and tear resistance as produced by summerwood fibers and at the same time a better appearance, a smoother surface and increased printability as produced by springwood fibers. These characteristics can all be achieved by my invention in connection with the use of two head boxes on a paper machine. Pulp consisting essentially of summerwood fibers is run through the primary head box to produce the body of the paper, and pulp consisting essentially of springwood fibers is run through the secondary head box to lay the springwood fibers on the surface of the paper being formed on the Fourdrinier wire, thereby achieving the combination of desired results.

Other applications and advantages may be achieved by fractionating the pulp according to the invention and using the separated fractions separately to make paper of differing grades on separate paper machines in the paper mill. Still other advantages may be achieved as by combining the fractions in predetermined proportions to make paper of a predetermined grade under controlled conditions.

It is obvious that much greater control of paper grade and characteristics can be achieved with decreased necessity for selection and control of the pulpwood used to make the pulp.

The practice of the present invention may be carried on with pulp at various consistencies and the consistency is not critical.

The fractionation is accomplished on the pulp after the pulp wood has been de-fiberized and thereby prepared

in the pulp slurry state. The process is applicable to pulp de-fiberized in any manner, including the chemical, semi-chemical and groundwood processes.

Specific examples of a process according to the invention, including the operative conditions and test results are as follows:

#### EXAMPLE I

A sample of pine kraft pulp was diluted to 0.10% consistency and pumped through a 3-inch Bauer centricleaner at 20 gallons per minute with 40 p.s.i. inlet pressure and zero outlet pressure. A minimum sized,  $\frac{1}{8}$  inch tip was used at the reject (bottom) discharge. The first separation produced 40% accepted (top) pulp and 60% rejected pulp.

The accepted and rejected pulps were each then pumped through the cleaner two more times under the same conditions as previously. In the second and third passes, the undesirable portions (rejects in the accepted pulp and accepts in the rejected pulp) were discarded. The final reject portion was defloured by pumping onto a 60 to 40 mesh screen which was the same that had been used to collect the accepted pulp. The approximate amounts of pulp obtained in each fraction after the three passes are as follows:

| Original                 |                   |         |         |
|--------------------------|-------------------|---------|---------|
| Weight, lbs. centrifuged | 78 lbs. (approx.) |         |         |
| First Pass               | Accepts           | Rejects |         |
| Weight, lbs. centrifuged | 31                |         | 47      |
| Percent                  | 40                |         | 60      |
|                          |                   |         |         |
| Second pass              | Accepts           | Rejects | Accepts |
| Weight, lbs. centrifuged | 22                | 9       | 10      |
| Percent                  | 71                | 29      | 21      |
| Percent of original      | 28                |         | 37      |
|                          |                   |         |         |
| Third pass               | Accepts*          | Rejects | Accepts |
| Weight, lbs. centrifuged | 19                | 3       | 4       |
| Percent                  | 86                | 14      | 11      |
| Percent of original      | 24                |         | 33      |

The final, asterisked accepted and rejected portions were evaluated for strength and fiber classifications in comparison with the original pulp. Table I shows the data obtained to be as follows:

The results in Table I show that a definite separation with respect to fiber characteristics was obtained. The accepted pulp had the characteristics normally attributed to springwood fibers and the rejected pulp resembled thick walled summerwood fibers. Compared to the original pulp, the accepted pulp had 17% higher mullen and 42% lower tear and the rejected pulp had 14% lower mullen and 39% higher tear. In addition, the accepted pulp had higher apparent density, smoothness, air resistance reading, fold and tensile than the rejected pulp. Further, fiber classifications showed that the accepted pulp had about 10% more long fibers (14 and 30 mesh) than the rejected pulp. Both fractions had more long fibers than the original pulp which was probably due to some loss of short fiber on the collecting screens and during deflouring.

#### EXAMPLE II

During the work covered by Example I, remarkably good separation of the springwood and summerwood components of pine kraft pulp was realized using a three-inch Bauer centricleaner and multiple passes at 0.1% consistency. Pulps with widely different strength characteristics were developed. However, such work showed that, if the same conditions were used on a paper mill scale, the power requirements for pumping would be very large. Consequently, further work was conducted to determine the degree of separation that could be obtained at higher consistencies and fewer passes. The data collected in this work are set forth in Table II.

The sample investigated was unbleached pine kraft pulp, portions of which were diluted to the selected consistencies (0.1% to 0.5%) and pumped only once through a three-inch Bauer centricleaner at 20 gallons per minute with 40 p.s.i. inlet pressure and zero outlet pressure and zero outlet pressure. A minimum sized, one-eighth inch tip was used at the reject (bottom discharge). The centricleaner separated pulp at a consistency of 0.1% to give 49% accepted pulp (top, springwood fraction) and 51% rejected pulp (bottom, summerwood fraction). At a consistency of 0.5%, the accepted portion was 74% and the rejected portion was 26%. These and other data collected during this work are included in Table II, infra, and, from them, it has been calculated that the pumping requirements for 100 A.D. tons of whole pulp per day at 0.1% consistency would be 15,000 gallons per minute with a head of at least 40 p.s.i.

Table I

| Sample                                      | Original    |        |        | Accepts*    |        |        | Rejects*    |       |       |
|---------------------------------------------|-------------|--------|--------|-------------|--------|--------|-------------|-------|-------|
|                                             | 21.4<br>733 |        |        | 21.2<br>727 |        |        | 21.0<br>758 |       |       |
| C.S. freeness                               | 500         | 400    | 300    | 500         | 400    | 300    | 500         | 400   | 300   |
| Power factor (kg.-min./cc.)                 | 1.43        | 1.18   | 0.99   | 1.79        | 1.42   | 1.11   | 1.49        | 1.24  | 1.09  |
| Beating factor (kg.-min.)                   | 320         | 371    | 413    | 360         | 413    | 473    | 364         | 430   | 494   |
| Mullen (percent, pt./lb.)                   | 145         | 149    | 151    | 167         | 173    | 179    | 120         | 127   | 134   |
| Tear factor                                 | 141         | 136    | 133    | 82          | 80     | 79     | 199         | 192   | 181   |
| Apparent density (lb./pt.)                  | 10.4        | 10.5   | 10.6   | 12.2        | 12.5   | 12.7   | 9.9         | 10.1  | 10.3  |
| Smoothness (sec./5 cc.)                     | 33          | 39     | 45     | 66          | 76     | 85     | 20          | 27    | 33    |
| Air resistance (sec./100 cc.)               | 14          | 54     | 108    | 439         | 986    | 3030   | 5           | 10    | 82    |
| M.I.T. fold                                 | 664         | 699    | 765    | 689         | 720    | 759    | 450         | 539   | 607   |
| Tensile (lb./1 in. width)                   | 31.8        | 33.0   | 34.3   | 40.6        | 42.2   | 43.6   | 28.1        | 29.7  | 30.7  |
| Breaking length (meters)                    | 9,820       | 10,200 | 10,700 | 12,500      | 12,900 | 13,300 | 8,590       | 9,030 | 9,360 |
| Gurley stiffness (mg.)                      | 122         | 10.19  | 116    | 104         | 103    | 101    | 138         | 137   | 131   |
| Fiber classifications, percent retained on: |             |        |        |             |        |        |             |       |       |
| 14 mesh                                     |             |        |        |             |        |        | 74.6        |       | 56.0  |
| 30 mesh                                     |             |        |        |             |        |        | 17.8        |       | 28.4  |
| 50 mesh                                     |             |        |        |             |        |        | 5.2         |       | 11.0  |
| 100 mesh                                    |             |        |        |             |        |        | 1.0         |       | 3.6   |
| Percent fines                               |             |        |        |             |        |        | 1.4         |       | 1.0   |

| Consistency used, percent.                  | Weight of original pulp, g. | 0.1         |             | 0.2         |             | 0.3         |             | 0.4         |           | 0.5         |           |
|---------------------------------------------|-----------------------------|-------------|-------------|-------------|-------------|-------------|-------------|-------------|-----------|-------------|-----------|
|                                             |                             | 2,999       | 2,993       | 2,993       | 3,272       | 3,054       | 3,054       | 3,820       | 3,820     | 3,820       | 3,820     |
| Sample                                      | Original                    | A.<br>1,469 | R.<br>1,530 | A.<br>1,870 | R.<br>1,063 | A.<br>2,183 | R.<br>1,089 | A.<br>2,129 | R.<br>925 | A.<br>2,839 | R.<br>981 |
| Weight of separated pulp, g.                |                             | 49          | 51          | 64          | 36          | 67          | 33          | 70          | 30        | 74          | 26        |
| Percent of original pulp                    |                             |             |             |             |             |             |             |             |           |             |           |
| Brightness, percent G.E.                    | 17.8                        | 17.5        | 17.3        | 18.1        | 17.6        | 18.1        | 18.1        | 18.0        | 18.2      | 17.8        | 18.1      |
| Initial C.S. freeness, cc.                  | 722                         | 679         | 749         | 712         | 746         | 713         | 723         | 723         | 747       | 718         | 732       |
| G.S.F., cc.                                 |                             |             |             |             |             |             |             |             |           |             |           |
| Power factor (kg.-min./cc.)                 | 500                         | 1.30        | 1.21        | 1.08        | 1.31        | 1.30        | 1.46        | 1.59        | 1.58      | 1.62        | 1.64      |
| Beating factor (kg.-min.)                   | 300                         | 0.88        | 0.80        | 0.81        | 0.89        | 0.97        | 0.97        | 0.97        | 1.01      | 1.02        | 1.02      |
| Mullen (percent, pt./lb.)                   | 500                         | 267         | 212         | 243         | 261         | 290         | 284         | 300         | 315       | 331         | 316       |
| Tear factor                                 | 300                         | 366         | 297         | 351         | 351         | 400         | 386         | 402         | 420       | 437         | 419       |
| Apparent density (lb./pt.)                  | 500                         | 146         | 156         | 130         | 155         | 129         | 152         | 137         | 151       | 136         | 146       |
| Smoothness (sec./5 cc.)                     | 300                         | 153         | 165         | 143         | 162         | 141         | 161         | 147         | 157       | 144         | 158       |
| Air resistance (sec./100 cc.)               | 500                         | 128         | 100         | 152         | 117         | 153         | 128         | 143         | 129       | 140         | 130       |
| M.I.T. fold                                 | 300                         | 121         | 97          | 140         | 111         | 139         | 123         | 131         | 123       | 129         | 121       |
| Tensile (lb./1 in. width)                   | 500                         | 11.1        | 11.7        | 10.4        | 11.2        | 10.6        | 11.1        | 10.6        | 11.2      | 10.6        | 10.6      |
| Breaking lengths (meters)                   | 300                         | 11.3        | 12.0        | 10.7        | 11.4        | 10.8        | 11.4        | 10.9        | 11.6      | 10.9        | 11.1      |
| Gurley stiffness (mg.)                      | 500                         | 40          | 54          | 28          | 44          | 18          | 43          | 27          | 30        | 31          | 47        |
| Fiber classifications, percent retained on: |                             |             |             |             |             |             |             |             |           |             |           |
| 14 mesh                                     | 500                         | 37          | 64          | 10          | 55          | 30          | 41          | 28          | 62        | 28          | 54        |
| 30 mesh                                     | 300                         | 341         | 619         | 94          | 435         | 252         | 383         | 233         | 542       | 252         | 389       |
| 50 mesh                                     | 500                         | 513         | 356         | 472         | 561         | 473         | 526         | 487         | 717       | 508         | 469       |
| 100 mesh                                    | 300                         | 641         | 440         | 518         | 482         | 651         | 657         | 557         | 591       | 577         | 503       |
| Percent fines                               | 500                         | 10,280      | 11,720      | 9,320       | 10,770      | 9,470       | 11,010      | 9,630       | 10,470    | 10,060      | 10,760    |
|                                             | 300                         | 11,020      | 12,650      | 10,390      | 11,310      | 9,980       | 11,470      | 10,710      | 11,160    | 10,870      | 11,650    |
|                                             | 500                         | 134         | 120         | 133         | 114         | 138         | 144         | 130         | 117       | 118         | 140       |
|                                             | 300                         | 126         | 117         | 128         | 108         | 131         | 130         | 126         | 116       | 119         | 126       |

The separation obtained with one pass through the centricleaner was not as pronounced as that reported in Example I, where each fraction was passed through the centricleaner two additional times and the undesirable portions were discarded. However, the results indicate that a definite separation with respect to fiber characteristics was obtained at each condition investigated. Compared to the original pulp at the 300 cc. freeness level, the accepted pulp, designated "A" in the columns of Table II, prepared at 0.1% consistency had 8% higher mullen and 20% lower tear, while the rejected pulp, designated "R" in the columns of Table II had 7% lower mullen and 16% higher tear. At 0.5% consistency, the accepted pulp (A) had 3% higher mullen and the same tear as the original pulp, while the rejected pulp (R) had 3% lower mullen and 5% higher tear. In every case, the accepted pulp had higher apparent density, smoothness, air resistance, fold, and tensile than the rejected pulp. When the consistency was increased, the difference in the tow fractions became less. There was no difference in the brightness of accepted and rejected pulp, but fiber classification showed that the accepted pulp had up to 10% more long fibers (14 and 30 mesh) than the rejected pulp.

I claim:

1. The process which comprises de-fiberizing wood into cellulosic pulp as an aqueous slurry containing a heterogeneous mixture of springwood and summerwood fibers, separating the mixture into fiber fractions respectively containing predominantly springwood and summerwood fibers by subjecting the slurry to forces which cause the fibers having a comparatively lower apparent specific gravity to separate from the fibers which have a comparatively higher apparent specific gravity, then making a paper-like sheet from at least one of the fiber fractions.

2. The process as set forth in claim 1 in which the slurry is subjected to centrifugal forces by treatment in a centrifugal separator.

3. The process as set forth in claim 1 in which the slurry is subjected to forces which cause the fibers to separate by sedimentation.

4. The process which comprises de-fiberizing wood into cellulosic pulp as an aqueous slurry containing a heterogeneous mixture of springwood and summerwood fibers, treating the slurry in a centrifugal separator to separate the mixture into fiber fractions respectively containing predominantly spring wood and summerwood fibers of comparatively lower and higher apparent specific gravity, then making a paper-like sheet by re-combining the pulp fractions in a predetermined manner.

5. The process which comprises de-fiberizing wood into cellulosic pulp as an original aqueous slurry containing a heterogeneous mixture of springwood and summerwood fibers, separating the slurry into at least two intermediate fractions the fibers of which respectively have predominantly higher and lower apparent specific gravities than the average specific gravity of the fibers in the original slurry and repeating at least once the said separation with respect to at least one of the intermediate fractions and forming a paper-like sheet from at least one of the end fractions thereby obtained.

#### References Cited in the file of this patent

#### UNITED STATES PATENTS

- |           |          |                |
|-----------|----------|----------------|
| 1,500,208 | Shaw     | July 8, 1924   |
| 1,818,897 | Kumagawa | Aug. 11, 1931  |
| 1,927,361 | Edge     | Sept. 19, 1933 |
| 1,951,017 | Hatch    | Mar. 13, 1934  |
| 2,972,171 | Heritage | Feb. 21, 1961  |